

Aug. 8, 1933.

G. S. VAN VOORHIS

1,922,020

ELASTIC WEBBING AND METHOD OF MAKING SAME

Filed Jan. 19, 1931



*Fig. 1*

*Fig. 2*



INVENTOR  
George S. Van Voorhis,  
BY  
J. W. Clegg,  
his ATTORNEY.

Patented Aug. 8, 1933

1,922,020

# UNITED STATES PATENT OFFICE

1,922,020

## ELASTIC WEBBING AND METHOD OF MAKING SAME

George S. Van Voorhis, Littleton, Mass., assignor  
to United Elastic Corporation, Easthampton,  
Mass., a Corporation of Massachusetts

Application January 19, 1931. Serial No. 509,625

5 Claims. (Cl. 91—68)

This invention relates to elastic sheet materials and to methods of making such materials.

Elastic fabrics of the kind commonly used in corsets, supporters, elastic stockings, and the like, are usually made by the weaving process, the rubber strands which give the elasticity to the fabric being woven into the goods while under tension, as is well understood by those skilled in this art. Such fabrics are necessarily relatively coarse and 10 they have a surface which is very objectionable to many people.

The present invention deals particularly with this difficulty. It aims to improve elastic fabrics with a view to making them more comfortable 15 to wear and giving them more pleasing surface characteristics. While the invention is especially concerned with fabrics, it is also contemplated that some features of the invention may be used to advantage in other forms of elastic sheet materials.

The nature of the invention will be readily understood from the following description when read in connection with the accompanying drawing, and the novel features will be particularly 25 pointed out in the appended claims.

In the drawing,

Figure 1 is a diagrammatic view illustrating certain steps of the method provided by this invention; and

30 Fig. 2 is a sectional view on a large scale of a piece of fabric embodying features of this invention.

Briefly stated, the invention involves the coating of any desired portion of the fabric with loose fibre, permanently attached to the fabric, the fibres of the coating preferably being so closely associated that they form a compact covering for the surface of the entire coated area.

According to the preferred method the fabric 40 is stretched or tensioned, a suitable adhesive such as rubber latex, rubber cement, or the like, is applied to the portion of the tensioned webbing which is to be coated, the fibre is dusted into this coating, and the coating is then allowed to dry, 45 the webbing being maintained under tension until the drying operation has proceeded to such a point that the goods will not be adversely affected by relieving the tension.

The apparatus used in practicing this method 50 may be of any suitable form. In the particular arrangement shown in Fig. 1 the webbing W is drawn from a supply roll 2 and is run between upper and lower feed rolls 3 and 4, respectively, which grip the fabric securely, both rolls being driven. The fabric travels over a table or sup-

port 5 to another pair of rolls 6 and 7 similar to the rolls 3 and 4. The rolls 6 and 7 also grip the fabric and are positively driven so that they feed the fabric, the web finally travelling from the lower roll 7 to the winding roll 8 where it is wound up on a suitable arbor or core 9. That section of the fabric between the two pairs of rolls is held constantly in a stretched or tensioned condition. As the web moves across the table 5 the rubber latex, rubber cement, or other adhesive, is applied to the surface of the webbing, for example, by spraying, as indicated at 10. This adhesive material may be applied in other ways, however, as for example, by rolling it on the fabric or in a spreader. Immediately after the application of the adhesive material the fibre is dusted on to the adhesive coating. The nature of the fibre used will depend upon the characteristics of the particular surface finish desired. Usually, however, a very short fibre will be used, 60 such as that known commercially as "flocks". This fibre is exceedingly short but different lengths are available, and flocks of various materials also can be readily obtained, such as cotton flocks, silk flocks, and the like. It may be 65 blown into the adhesive coating on the webbing W through a nozzle 12, Fig. 1, or it may simply be shaken on to the webbing, or it may be applied 70 in any other suitable manner.

After the application of the flocks a suitable 75 interval preferably is allowed for the adhesive coating to dry before the fabric reaches the rolls 6 and 7, and the drying operation may be hastened in any desired manner, as for example, by passing it under a suction hood 14 or over a 80 warm plate 15, or the like.

The surplus flock or fibre can be removed at 85 any desired point, either during the process just described or at a subsequent operation. It is also contemplated that the fabric will be subjected to additional finishing operations of a 90 character to be determined by the requirements of individual cases.

According to the preferred process, as above indicated, the web W is maintained in a stretched 100 and tensioned condition during the application of the adhesive, the dusting operation, and until the drying has proceeded to the desired point. This produces a denser association of the fibres, a more complete coating of the surface, and a 105 more compact fibrous coating.

In Fig. 2 the rubber strands of fabric are indicated at 16, the strands being interwoven with the warp and filling threads or yarn in the usual manner, and the fibre coating is shown at 17. 110

It may here be pointed out that the individual fibres of this coating are independent of each other except insofar as they are all adhesively secured to the fabric by the adhesive. The fibres, 5 however, are not interlocked with each other and have no association independent of their union to the fabric as would be the case if they formed a part of a separate fabric. Consequently, the elasticity of the fabric is not affected in any manner 10 by the coating.

The fabric so produced has surface characteristics quite unlike those of the ordinary elastic fabrics. The surface is soft and pleasing to the touch as distinguished from the relatively harsh 15 feel of elastic webbing of the more common kinds. The surface appearance also is quite different. This fabric, therefore, is far more suitable for use in many garments and articles of apparel. While it is less porous than ordinary 20 webbing, this fact is an advantage for some purposes, as in reducing garments. The adhesive coating is also of advantage in reducing the tendency of the fabric to fray or ravel when cut, and providing a more secure union when sewed 25 to another part of a garment. The application of the latex, rubber cement, rubber dispersion, or the like, to the elastic fabric while it is under tension ensures a sufficient penetration of the 30 latex into the fabric to bond the rubber coating to the strands of rubber and the threads of which the elastic fabric is composed. Consequently, when the finished fabric is cut it will be found that the rubber warps and the thread filling are 35 so bonded together that the fabric will neither ravel, nor will the strands of rubber warp contract and pull the ends back into the body of the fabric away from the cut surface, as is usual in the ordinary forms of woven rubber webbing.

As this material is largely used in the manufacture 40 of corsets, a great many times in panel form, the process described makes it possible to sew these panels into the corset and they will not pull out as is often the case. For some purposes the flocks or fibre is not necessary and will 45 not be used.

Other forms of elastic sheet materials, as for 50 example sheet rubber, can be treated in essentially the same manner to give it a softer and more agreeable surface, as distinguished from the cold and somewhat tacky surface characteristic of rubber.

While I have herein disclosed a preferred embodiment of my invention, it will be understood that the invention may be embodied in other forms without departing from the spirit or scope thereof.

Having thus described my invention, what I desire to claim as new is:

1. That improvement in methods of manufacturing elastic sheet material formed at least partially of rubber, which consists in stretching 85 said material, and, while holding the material so stretched and elongated, adhesively securing a coating of short loose fibre to the surface thereof, to provide a flocked surface.

2. That improvement in methods of manufacturing elastic sheet material formed at least partially of rubber, which consists in coating the surface of the material with an adhesive, applying loose fibre to said adhesive while it is in a sticky 95 condition whereby a coating of said fibre will be united to the material, and holding the material in an elongated condition and under tension while performing said operations and while said adhesive dries.

3. That improvement in methods of manufacturing elastic sheet material formed at least partially of rubber which consists in applying to the surface of said material a coating of a rubbery adhesive, dusting loose fibre into said adhesive while it is in a sticky condition, and holding the 105 material in an elongated condition and stretched while said coating and dusting operations are performed and while the adhesive dries.

4. That improvement in methods of manufacturing elastic webbing of rubber and textile material which consists in stretching the webbing and thereby elongating it, applying and adhesively uniting a coating of flocks to said webbing while it is held so stretched and elongated, thereby to provide a flocked surface on the web- 110 115 bing.

5. That improvement in methods of manufacturing elastic webbing of rubber and textile material which consists in stretching the webbing, applying adhesive to the surface of the webbing, 120 dusting flocks into said adhesive while it is in a sticky condition, and holding the webbing stretched and elongated during the said applying and dusting operations and until the adhesive has substantially dried.

GEORGE S. VAN VOORHIS.